

# UNITED STATES PATENT OFFICE.

CHARLES HENRY PHILLIPS, JAMES TRODEN, AND JOHN GOLLING, OF ALPENA, MICHIGAN.

## FIRE AND WATER PROOF PAINT.

SPECIFICATION forming part of Letters Patent No. 326,776, dated September 22, 1885.

Application filed June 23, 1885. (No specimens.)

*To all whom it may concern:*

Be it known that we, CHARLES H. PHILLIPS, JAMES TRODEN, and JOHN GOLLING, citizens of the United States, residing at Alpena, in the county of Alpena and State of Michigan, have invented certain new and useful Improvements in Fire and Water Proof Paint, of which the following is a specification.

Our invention relates to an improved paint compound especially adapted for covering roofs, damp walls, or any surface where a fire and water proof paint is desirable.

Our paint consists of the following ingredients, combined in about the proportions set forth, namely: one barrel of tar, ten pounds red mineral, ten pounds keystone granite, ten pounds water-lime, eight pounds asbestos, ten pounds potash, and ten pounds alum.

The tar should be boiled for about two hours, or until the gas has all escaped. The other components are then added to the tar, one at a time, in the order named, and while the latter is at the maximum heat, and the mixture boiled one hour, during which time it should be frequently stirred. It should be applied to wood—shingles, for instance—in its hottest condition—say, while at a temperature of 220°

Fahrenheit. In applying it to tin or iron surfaces the temperature may be less—say, 200° Fahrenheit.

The proportions herein named have been ascertained by careful experiment and are deemed to produce the best results; but said proportions may be varied somewhat without departing from the invention.

Made and applied as here described the paint produces a coating that will resist the ordinary action of both fire and water, and it is unaffected also by cold. It will not scale off.

Having described our invention, we claim and desire to secure by Letters Patent of the United States—

A paint compound consisting of tar, red mineral, keystone granite, lime, asbestos, potash, and alum, combined substantially in the proportions set forth.

In testimony whereof we affix our signatures in presence of two witnesses.

CHARLES HENRY PHILLIPS.

JAMES TRODEN.

JOHN GOLLING.

Witnesses:

GEO. H. SLEATOR,

WM. T. SLEATOR.